

## UNITED STATES PATENT OFFICE.

CHARLES B. JACOBS, OF WILMINGTON, DELAWARE, ASSIGNOR TO E. I. DU PONT DE NEMOURS & COMPANY, OF WILMINGTON, DELAWARE, A CORPORATION OF DELAWARE.

## CASTING HAVING SILICON-ALLOY SURFACE.

No Drawing.

Application filed April 30, 1921. Serial No. 465,686.

This invention relates to ferrous metal castings the surface portions of which are alloyed with silicon, and it comprises, as a new process, the forming of an alloy surface on the casting during the casting operation, and, as a new article of manufacture, a ferrous metal casting, such as cast iron and cast steel, the surface portion of which is alloyed with silicon to such an extent as to substantially increase the resistance of said surface portion to corrosion, and especially to the corrosive action of acids.

I have discovered that a casting, in which a surface portion, or layer, thereof is alloyed with a comparatively large proportion of silicon, can be produced by bringing the casting metal into contact with suitably sub-divided silicon or ferrosilicon during the casting operation, provided certain conditions with respect to temperature and composition of the casting metal are observed.

Generally speaking, my new method comprises coating those surfaces of the mold or cores of the mold in which the casting is made, corresponding with the surfaces of the casting on which the alloy is required, with silicon or ferrosilicon in a granular condition in such a manner that the casting metal on flowing into the mold does not wash the metallic coating from the coated surfaces, but when poured into the mold at the proper temperature flows over and melts or dissolves the metallic coating. The "skin-chill" or chilling effect exerted by the mold surfaces prevents the silicon from diffusing throughout the body of the casting metal so that an alloy is formed on the surface of the casting containing a high percentage of silicon.

To prevent the coating from being washed from the mold surfaces by the flow of the casting metal, the silicon in a granular or comminuted condition is mixed with a suitable binder into a plastic mass and applied to the mold or core surfaces and then dried so that it adheres firmly to the surfaces, forming a coating containing spaces filled with binder between the silicon granules. When poured into the mold, the molten casting metal enters and displaces the binder from said spaces and melts or dissolves the metallic particles.

It is important to apply the coating evenly all over the mold or the core surfaces, as the case may be, in such physical condition that the granules of silicon or ferrosilicon shall have spaces therebetween into which the casting metal may enter after displacing the binder. For this reason it is necessary to make the size of the granules such that the spaces between the granules will be sufficiently large to permit the proper quantity of the particular casting metal to enter and melt or dissolve the silicon. When granulation has been carried too far and the coating metal contains a considerable proportion of materials of an extreme degree of fineness, say, from 40 to 100 mesh and finer, the coating does not furnish voids large enough to permit the casting metal in sufficient volume to surround the particles of the coating metal and dissolve or melt it. An example of the effect of the coating material in too fine a state of granulation may be cited in the case of ferrosilicon and cast iron.

When the mold was coated with ferrosilicon showing the following sizing test,—material passing through 18 mesh retained on 30 mesh screen 35% by wt., material passing through 30 mesh retained on 60 mesh screen 37% by wt., material passing through 60 mesh 28% by wt.—the voids of the coating were not large enough to allow sufficient iron to enter and surround the particles of ferrosilicon, consequently the iron running into the mold dissolved only a thin skin surface of the coating and the casting produced had only a very thin layer of ferrosilicon on its surface which was not continuous as there were spots where the iron had failed to dissolve any ferrosilicon. On the other hand when the mold was coated with ferrosilicon sized to between 18 and 30 mesh, made into a plastic mass with the same binder used with the finer material, the finished casting poured at the same temperature, contained an alloy high in silicon from its surface to the depth of  $\frac{1}{4}$ " below the surface.

The new method as applied to cast iron may be advantageously practiced with silicon or ferrosilicon particles having a size between 15 and 35 mesh, that is, all of the particles passing through a 15 mesh screen

and substantially all of the particles being caught on a 35 mesh screen.

Steel on account of its freedom from the relatively large amount of impurities which go to make up cast iron takes silicon into solution more readily than does cast iron, so that it is desirable to use more finely divided particles of silicon or ferrosilicon than in the case of cast iron, particles sized, for example, between 20 and 60 mesh.

In surfacing cast iron with silicon according to my invention it is necessary to raise the temperature of the cast iron above the melting point of the silicon in order to obtain a true alloy on the surface of the iron. Pure crystallized silicon melts at 2588° F. and ferrosilicon at a somewhat lower temperature, depending on the percentage of silicon it contains. A mold coated with ferrosilicon containing about 81% silicon, was poured at the ordinary temperature at which iron castings are usually poured, i. e., about 2600° F. or slightly above. The metal failed to take up more than a thin coating of silicon and this coating when examined under the microscope, showed that the greater part of the silicon was composed of particles embedded in a matrix of iron, still retaining their identity, as marked by their crystalline structure. However, when the iron was raised to a temperature of 2700 to 2800° F. and then poured, the silicon was taken into solution in the iron and a true silicon alloy formed on the surface of the casting. Cast steel on the other hand readily takes silicon into solution at a temperature below 2600° F. There are also other conditions necessary for the successful formation of silicon alloys on cast iron and cast steel that will be described hereinafter.

The depth to which the alloy penetrates below the surface of the casting is very largely dependent on the thickness of the coating of the mold or core surfaces and in a general way except for slight general diffusion, the depth of penetration corresponds approximately with the thickness of the coating on the mold. This varies with the thickness and nature of the casting. Molds for heavy castings of thick sections which cool slowly may be coated to a depth of  $\frac{1}{4}$ " and even greater, while molds for light castings of thin sections which cool rapidly may only be coated to a limited depth (about  $\frac{1}{16}$ " to  $\frac{1}{8}$ ") in order that the casting metal may have time to dissolve or melt the entire coating before the casting metal begins to solidify. If the coating of the mold is too thick the resulting casting will have a pitted uneven surface with a large part of the coating metal not forming a true alloy but simply embedded in a matrix of the casting metal.

It is obvious that alloys may be formed on the inside surface of hollow castings as well as on the outside of the casting and that

these alloys may be of the same character or of entirely different character on the same casting, as for example, chromium on the outside surface of an iron or steel casting to resist oxidation at high temperature and silicon on the inside surface to resist corrosion by acids.

Ferrous metal castings on account of their strength and cheapness offer the largest commercial field for this process. When alloyed with the proper metal or alloy to render them resistant to corrosion by liquids or gases they serve to replace the brittle and comparatively expensive high silicon alloys containing from 12 to 18% of silicon used as acid-resistant metals.

My invention may be explained in more detail as follows, reference first being had to the surfacing of cast iron with silicon.

The molds to be used are the ordinary green sand molds either blackened or untreated in which iron castings are usually made. The silicon made into a paste with sodium silicate solution is applied to the mold or core surfaces and dried; baking of the mold is not necessary, ordinary skin drying being all that is required for cast iron. A coating  $\frac{1}{8}$ " thick, made from sodium silicate solution and ferrosilicon in suitable proportions, will contain about 1 lb. of metallic silicon per square foot.

In forming alloys high in silicon on the surface of cast iron for resistance to acid it was found that when the iron was poured at the ordinary temperature at which iron castings are usually poured, i. e., about 2500-2600° F., the metal failed to take up more than a thin coating of silicon and this coating when examined under the microscope showed that the greater part of the silicon grains were embedded in a matrix of iron and still retained their identity as marked by their crystalline structure and general contour. By the use of thermit introduced into the ladle of metal after it had been tapped from the cupola it was possible to raise the temperature of the cast iron to between 2800 and 2900° (pyrometer measurements). When the metal was poured into the molds surfaced with silicon or ferrosilicon at this temperature the iron melted the silicon and took it into solution. The "skin chill" of the mold prevented any great amount of diffusion of the silicon in the iron so that an alloy high in silicon was built up on the surface of the casting to a depth corresponding substantially with the thickness of the silicon coating on the mold surfaces, i. e., about  $\frac{1}{8}$ " on small castings and  $\frac{1}{4}$ " on larger castings.

I also found that if the silicon with which the mold was coated was too finely divided, as before pointed out in the general discussion, it left such small voids between the particles in the coating that the free caustic

soda in the commercial sodium silicate (about 10%) acted on the finely divided silicon when the coated surface of the mold was heated to skin dry it, and cemented the whole coating together with silicate of soda leaving no voids for the melted iron to enter, consequently the iron running in the mold dissolved only a thin skin surface of the silicon coating and the casting came out of the mold with only a very thin layer of ferrosilicon on its surface which was not continuous as there were spots where the iron had completely failed to fix any perceptible amount of silicon. It was first thought that the failure of iron to take up finely divided silicon was due to the action of the free caustic in the silicate of soda solution. The caustic in the solution was therefore neutralized with boric acid. However, when the silicon was too finely divided the same general effect was obtained with the use of neutralized sodium silicate and also with the use of "Glutrin" binder (a product used in foundries for making cores and containing no caustic soda) as with unneutralized sodium silicate, and while this action was accentuated by the presence of the caustic soda, the behavior of too finely divided silicon in the coatings showed that in order to obtain a uniform alloy high in silicon on the surface of the casting it is necessary to maintain a certain degree of porosity in the coating of the mold by using silicon particles of the proper size so that the iron can run into the voids and surround the particles of the silicon or ferrosilicon while it is at a temperature sufficiently high to melt or take the silicon into solution.

Silicon or high ferrosilicon sized to from 18 to 30 mesh and made plastic and adhesive to the mold or core surfaces with 40° Bé. silicate of soda solution mixed 1 to 1 with water is what I prefer to use.

Another feature developed by the attempts to build up a high silicon alloy on the surface of cast iron was the action of the silicon on the carbon in the iron. Ordinary cast iron contains from 3.5 to 4% of total carbon, mostly in the graphitic condition. A high percentage of silicon in the melted iron has the effect of throwing carbon out of solution in the form of graphite so that, when ordinary cast iron is used on molds coated with silicon or ferrosilicon, sections cut from the castings, poured at a sufficiently high temperature to obtain actual melting or solution of the silicon in the iron, show a band of demarcation containing more or less graphite carbon segregated between the high silicon area (which has been formed on the face of the castings) and the underlying cast iron area.

In large castings of thick sections requiring a considerable time to solidify or set, the separated graphite may even become dis-

seminated through the high silicon and to a sufficient extent to introduce a certain degree of porosity in the high silicon alloy itself. Such castings while much more resistant to corrosion by acids than ordinary cast iron are not entirely satisfactory as absolutely acid proof castings, since slow seepage of acid is likely to occur through the porous graphite, if present in considerable quantity, and eventually reach the body metal below the high silicon area.

In small castings or castings with thin sections which cool rather quickly this effect of the silicon on the separation and segregation of graphite is less marked and in most cases will not induce porosity in the high silicon area of the casting.

The undue separation of graphite by the action of the high silicon content of the melted iron and the ill effects noted above may be minimized to such an extent as to be harmless by conducting the casting operation under the proper conditions. In castings having thick sections in which the metal requires too long a time to freeze or set, the separation of graphite may be lessened by placing "chills" or pieces of metal in the mold opposite these sections to conduct the heat away more rapidly and induce freezing or settling of the metal while it still retains its graphite content evenly distributed.

Carbon-free ferromanganese which has the power of absorbing and holding a large amount of carbon in the combined state may be added to the iron in the ladle to absorb and hold the carbon from separation as graphite induced by the action of the silicon.

The separation of graphite from the melted iron can also be avoided by partially decarburizing the iron to a point where it will retain its graphite on cooling, evenly distributed through the structure of the iron by adding sufficient low carbon steel scrap to the cupola and ladle to lower the carbon content of the iron to prevent the separation of graphite. When steel scrap is added to the ladle as well as to the cupola it is usually necessary to use thermit in the ladle to help melt the steel and keep the iron sufficiently fluid to pour properly.

Decarburization of the iron can be accomplished by introducing the iron tapped from the cupola into a small Bessemer converter and blowing it for a sufficient time to partially burn out its carbon content. If decarburized to a sufficient extent the metal will have substantially the same carbon content as steel but, unlike steel, will still contain most of the impurities existing in cast iron.

Operating under the proper conditions above indicated, satisfactory high silicon alloys resistant to corrosion by various gases and liquids may be formed on the surface of cast iron.

The character of the silicon alloy formed

with a body metal of gray cast iron is indicated by the percentages of silicon, given in the following table, at various distances from the face of the casting:

| Location of sample.                               | Per cent silicon. |
|---------------------------------------------------|-------------------|
| 1. Surface layer $\frac{1}{8}$ " thick            | 32.57             |
| 2. Drillings $\frac{3}{8}$ " from face of casting | 2.68              |
| 3. " $1\frac{1}{8}$ " " " "                       | 2.56              |
| 4. Gray cast iron (analysis of test bar)          | 2.39              |

A comparison of the analytical results given above with the results published by S. J. Tungay in *Jour. Soc. Chem. Ind.* Vol. 37, page 87 (1918) which show the influence of the silicon content in ferrosilicon to 10% hydrochloric, nitric, and sulphuric acids respectively, makes it evident that the alloy on the surface of the casting, and to a depth of at least  $\frac{1}{8}$ " below the surface, possesses the maximum resistance to the corrosive action of the above-mentioned acids.

Microscopic examination of sections cut from the casting on a line perpendicular to the alloyed surface also shows the gradation of the high silicon alloy on the surface of the casting into the cast iron body below. The samples were polished in the usual manner and then etched for 15 seconds with a solution prepared by adding 4 cc. of nitric acid, sp. gr. 1.42 to 96 cc. of 95% grain alcohol. The high silicon area was found to extend to a depth of  $\frac{1}{4}$  of an inch from the edge of the sample indicating that the silicon content to this depth was above 10%.

In addition to being resistant to acids castings made according to my invention have all of the inherent strength of gray cast iron by virtue of the underlying body metal, whereas ferrosilicon containing as little as 14% of silicon cannot be machined, is so weak and brittle as to narrowly limit the size and shape of castings into which it can be formed, and has such high shrinkage that castings thereof are frequently marred by checks and cracks. By my invention silicon alloys may be formed on, and to a considerable depth below, the surface on any casting that may be made of gray cast iron irrespective of size or shape.

In forming silicon alloys on cast steel, the preparation of molds, application of the silicon or ferrosilicon, and the use of binders is substantially the same as in the case of silicon on cast iron. The casting operation however should be conducted at a much lower temperature than was used for silicon on cast iron and certain precautions must be observed before high silicon alloys can be built up on the surface of cast steel.

Silicon is much more soluble in steel than in cast iron and when taken into solution in the steel lowers the melting point of the

metal to a marked degree so that while remaining at the same temperature, steel to which silicon has been added becomes much more fluid and requires a longer period to freeze or set. This well known effect of silicon in lowering the melting point of steel is taken advantage of in the open hearth steel process of making low carbon steel for casting purposes. The same increased fluidity is produced in the steel 70 poured into a mold coated with silicon or ferrosilicon. The metal while remaining at the same temperature is so much more fluid that it requires a longer cooling period to reach its freezing or setting point, and unless precautions are taken to increase the rate of cooling, lower the temperature of the casting metal, or slow up the rate of solution of the silicon in the steel, diffusion of the dissolved silicon will take place 80 throughout the steel before the chilling effect of the ordinary mold surfaces can act to build up a high silicon alloy on the surface of the casting next the molds. For example steel from a heat of the following 90 analysis:

|             | Per cent. |
|-------------|-----------|
| Carbon      | .24       |
| Manganese   | .65       |
| Silicon     | .289      |
| Phosphorous | .038      |
| Sulphur     | .037      |

was poured into a mold for producing a casting 2" in thickness. The mold, coated on the face to a depth of  $\frac{1}{4}$  of an inch with 100 93% ferrosilicon sized to from 18 to 30 mesh, was taken from the baking oven at a temperature of 650° F. and immediately closed and cast. The temperature of the steel as it was poured into the mold was 2660° F. (i. e. about the usual temperature of pouring low carbon open hearth steel castings). An analysis of the face of the casting corresponding with the coated surface of the mold showed 1.75% silicon while the back of the casting showed 1.01% silicon. The silicon rapidly dissolved from the coated face of the mold and taken into solution in the incoming steel lowered the freezing point of the metal to such an extent that almost complete and uniform diffusion of the silicon took place throughout the whole body of the casting before the "skin chill" of the mold could solidify the metal entering the hot mold at 2660° F. and build up a high silicon alloy next the mold surfaces.

To successfully produce high silicon alloys on the surface of low carbon steel castings it is necessary to pour the casting at as low a temperature as it is possible to pour the metal and have it run to all parts of the mold in question. A temperature of 2600 or as much below that as the nature of the casting will permit usually gives good re-

sults, especially if the mold has been allowed to stand and cool to room temperature before the casting is poured.

In castings with thick sections where the metal would naturally cool slowly it is advisable when the nature of the casting will permit to set "chills", (i. e. blocks of steel) in the mold opposite these sections to increase the rate of cooling induced by the mold surfaces.

For steel castings, especially with low carbon steel, the silicon or ferrosilicon with which the molds are coated should be reduced to a much finer state of division than is the case with cast iron in order to furnish smaller voids for the steel to enter and thus slow up the rate of solution of the silicon in the steel. In the example pointed out above ferrosilicon sized to from 18 to 30 mesh gave quick solution and almost complete diffusion of the silicon throughout the whole area of the casting even when poured at a fairly low temperature. Silicon or ferrosilicon sized from 20 to 60 mesh and even finer offers smaller voids in the coating for the steel to enter and slows up the rate of solution sufficiently to enable the chilling effect of the mold to make itself felt before dissemination of the silicon throughout the body of the steel has occurred, with the result that an alloy high in silicon is built up next the mold surfaces.

Green sand molds skin dried but not baked may also be used to increase the chilling action of the mold surfaces and prevent too rapid diffusion of the silicon in the steel. The danger of porous castings which frequently occur when ordinary steel castings are made in green sand molds is obviated in this case by the tight, close-grained structure of the high silicon alloy on the surface of the castings next to the mold surfaces, and the skin drying of the mold surfaces.

Certain types of steel castings, the body metal of which it is desirable to make of soft easily machinable steel having a high silicon alloy on the surface, are frequently of such shape that they do not lend themselves to the method of using "chills" in the mold and of such a character, on account of thickness of section, etc., that the chilling effect of green sand molds alone does not sufficiently check the solution and diffusion of the silicon or ferrosilicon in the steel to cause the formation of a silicon alloy of the desired silicon content on the surface of the castings. With castings of this type I have found by practice that the desired result may be obtained by adding some form of active carbon to the silicon or ferrosilicon with which the mold surfaces are coated, as for example, finely divided willow charcoal. With castings of an inch in section from 10 to 15% of willow charcoal added to 80% ferrosilicon and made into a plastic mass

with silicate of soda solution for surfacing the molds gives the desired results. On castings of greater thickness of section, as for example, two inches or more in section, it is necessary to add a greater proportion of charcoal to the ferrosilicon. As much as from 20 to 30% has been found to give desirable results. Advantage is taken here of the well known fact that molten steel will dissolve a considerable amount of carbon in the form of charcoal. This same action takes place in the mold during the casting operation and the solution of the carbon in the steel slows up the solution and diffusion of the silicon, and causes the formation of a high silicon alloy on the surface of the casting. The penetration of the carbon in the steel is confined substantially to a depth corresponding to the depth of the coating of ferrosilicon and carbon on the mold surface.

Operating under the proper conditions and observing the precautions necessitated by the character of the casting in question, silicon alloys may be formed on the surface and to a depth of  $\frac{1}{4}$  of an inch and more below the surface of steel castings containing from 30 to 50% or more of silicon at the skin surface and grading off to low silicon content where the high silicon alloy merges into the steel body metal of the casting. Sections cut from such castings will show the same bonding of the high silicon area above and the cast steel below that is shown by chromium alloyed on cast steel. In the merging band and in the high silicon area no graphite will show as it did in the case of silicon and cast iron. The high silicon area composed of silicon and ferrite will show a close grained dense structure and the merging band will show traces of this structure together with the ferrite and pearlite of the underlying steel body metal of the casting.

Castings made by the formation of high silicon alloys on the surface of cast steel have the acid proof qualities of high ferrosilicon and the inherent strength of cast steel and can be made into shapes and sizes for resistance to acid not possible with ferrosilicon on account of its brittleness and lack of mechanical strength.

As has been indicated above, castings having the desired properties can be made starting either with pure silicon or with ferrosilicon. In practicing the invention on a commercial scale, pure silicon is eliminated as a starting material at the present time because of its high cost. The ferrosilicons which I prefer to use are those high in silicon, although the silicon content may vary within wide limits. As a rule a ferrosilicon having 75% or more of silicon gives good results.

As will be understood by those versed in the art to which this invention relates, vari-

ous changes in details may be made in the method above described without departing from the spirit and scope of my invention.

I claim:

- 5 1. The method of making a ferrous metal casting having a surface strongly resistant to the corrosive action of acids, which comprises coating a surface of the mold in which the casting is to be formed with a mixture 70  
10 of ferrosilicon particles having sizes between 15 and 40 mesh and a binder therefor, hardening the coating, and then introducing 75  
15 into said mold molten ferrous metal at a temperature at which substantially all of the particles of ferrosilicon will dissolve 80  
therein.
2. The method of making a ferrous metal casting having a surface strongly resistant to the corrosive action of acids, which comprises 85  
20 coating a surface of the mold in which the casting is to be formed with a mixture of ferrosilicon particles containing more than 75% of silicon and having sizes between about 15 and 35 mesh and a neutralized sodium silicate solution, drying the coating, and then introducing into said mold molten ferrous metal at a temperature at which said ferrosilicon particles will dissolve therein, said temperature being low enough to allow 90  
30 solidification to occur while the dissolved silicon is still concentrated near the surface of the casting.
3. The process of forming a silicon alloy 95  
25 on the surface of cast iron which comprises coating a surface of the mold in which the casting is to be formed with a mixture containing ferrosilicon particles and a liquid binder therefor, hardening the coating, and then introducing into said mold molten cast 100  
40 iron at a temperature above 2650° F., the size of said particles being such as to permit ready penetration therebetween by said molten cast iron.
4. The process of forming a silicon alloy 105  
45 on the surface of cast iron which comprises coating a surface of the mold in which the casting is to be formed with a mixture containing ferrosilicon particles and a liquid binder therefor, hardening the coating, and then introducing into said mold molten cast 110  
50 iron at a temperature of from about 2700 to 2900° F., the size of said particles being such as to permit ready penetration therebetween by said molten cast iron.
5. The process of forming a silicon alloy 115  
55 on the surface of cast iron which comprises coating a surface of the mold in which the casting is to be formed with a mixture containing ferrosilicon particles sized between about 120  
60 15 and 35 mesh and a liquid binder therefor, hardening the coating, and then introducing into said mold molten cast iron at a temperature of from about 2700 to 2900° F.
6. The process of forming a silicon alloy 125  
65 on the surface of cast iron which comprises coating a surface of the mold in which the casting is to be formed with a mixture containing ferrosilicon particles having more than 75% of silicon and sized between about 15 and 35 mesh and a binder for said particles capable of holding them on the surface of the mold, hardening the coating, and then introducing into said mold molten cast iron at a temperature sufficient to enable said iron to penetrate between, and dissolve, substantially all of said particles.
7. The process of forming a silicon alloy 80  
130 on the surface of cast iron which comprises coating a surface of the mold in which the casting is to be formed with a mixture containing ferrosilicon particles having more than 75% of silicon and sized between about 15 and 35 mesh and a binder for said particles capable of holding them on the surface of the mold, hardening the coating, and then introducing into said mold molten cast iron at a temperature of from about 2800 to 2900° F.
8. The process of making a steel casting 90  
135 having a silicon alloy surface, which comprises coating a surface of the mold in which the casting is to be formed with a mixture containing metallic particles comprising silicon of sizes between about 20 and 60 mesh and a liquid binder therefor, hardening said coating, and then introducing into said mold molten steel at a temperature near its solidifying point to permit solidification thereof before a major portion of the silicon which is dissolved thereby has become dispersed throughout the body of the casting.
9. The process of making a steel casting 100  
140 having a silicon alloy surface, which comprises coating a surface of the mold in which the casting is to be formed with a mixture containing finely divided ferrosilicon and a liquid binder therefor, hardening said coating, and then introducing into said mold molten steel at a temperature of 105  
145 from about 2575 to 2650° F.
10. The process of making a steel casting 110  
150 having a silicon alloy surface, which comprises coating a surface of the mold in which the casting is to be formed with a mixture containing comminuted ferrosilicon sized between about 20 and 60 mesh and a liquid binder therefor, hardening said coating, and then introducing into said mold molten steel at a temperature near its solidifying point to permit solidification thereof before a major portion of the silicon which is dissolved thereby has become dispersed throughout the body of the casting.
11. The process of making a steel casting 115  
160 having a silicon alloy surface, which comprises coating a surface of the mold in which the casting is to be formed with a mixture containing comminuted ferrosilicon 120  
165 sized between about 20 and 60 mesh and a liquid binder therefor, hardening said coating, and then introducing into said mold molten steel at a temperature of from about 2700 to 2900° F.

sized between about 20 and 60 mesh and having more than 75% silicon and a sodium silicate solution, hardening said coating, and then introducing into said mold molten steel at a temperature of from about 2575 to 2650° F.

12. The process of making a steel casting having an iron-silicon alloy surface in the form of a surface layer containing a large percentage of silicon, the body of the casting having a relatively small percentage of silicon, which comprises coating a surface of the mold in which the casting is to be formed with a mixture comprising carbon in a form readily soluble in molten steel, metallic particles comprising silicon, and a binder for said particles, allowing said coating to harden, and then introducing into said mold molten steel at a temperature at which the carbon will be effective to prevent the silicon in said coating from diffusing freely throughout the body of steel.

13. The process of making a steel casting having a silicon alloy surface, which comprises coating a surface of the mold in which the casting is to be formed with a mixture containing carbon in a form readily soluble in molten steel, ferrosilicon of sizes between about 20 and 60 mesh and a liquid binder therefor, hardening said coating, and then introducing into said mold molten steel at a temperature near its solidifying point to permit solidification thereof before a major portion of the silicon which is dissolved thereby has become dispersed throughout the body of the casting.

14. The process of making a steel casting having a silicon alloy surface, which comprises coating a surface of the mold in which the casting is to be formed with a mixture containing carbon in a form readily soluble in molten steel, finely divided ferrosilicon and a liquid binder therefor, hardening said coating, and then introducing into said mold molten steel at a temperature of from about 2575 to 2650° F.

15. As a new article of manufacture, a ferrous metal casting having silicon alloyed therewith at the surface, the silicon content decreasing from a value of more than 30% at the surface to a value of less than 10% at three-eighths of an inch from the surface.

16. As a new article of manufacture, a ferrous metal casting associated at its sur-

face with silicon, substantially all of said silicon being alloyed with the ferrous metal of the casting and constituting more than 20% of a surface layer one-eighth of an inch thick.

17. As a new article of manufacture, a cast iron casting having silicon alloyed therewith at the surface, the silicon content of a surface layer one-eighth of an inch thick being more than 20%, and the silicon content of the remainder of the casting being substantially less than 20%.

18. As a new article of manufacture, a cast iron casting having silicon alloyed therewith at the surface, the silicon content of a surface layer one-eighth of an inch thick being about 30%, and the silicon content of the remainder of the casting being substantially less than 20%.

19. As a new article of manufacture, a steel casting associated at its surface with silicon, substantially all of said silicon being alloyed with the steel of the casting, the silicon content being more than 20% at the surface and decreasing toward the interior.

20. As a new article of manufacture, a steel casting associated at its surface with silicon, substantially all of said silicon being alloyed with the steel of the casting, the silicon content being more than 20% at the surface and decreasing toward the interior, the alloy surface of the casting being obtainable by limited diffusion of silicon into the cast steel while the latter is in a molten condition.

21. As a new article of manufacture, a steel casting having silicon alloyed therewith at the surface, the body metal of the casting being of soft easily machinable steel, most of said silicon being concentrated in a surface layer of about one-quarter of an inch or less in thickness, and said surface layer having a substantially greater carbon content than has the body of the steel casting.

22. As a new article of manufacture, a steel casting having silicon alloyed therewith at the surface, the body metal of the casting being of soft easily machinable steel, most of said silicon being concentrated in a thin surface layer, and said surface layer having a substantially greater carbon content than has the body of the steel casting.

In testimony whereof I affix my signature.

CHARLES B. JACOBS.